

# UNITED STATES PATENT OFFICE.

JOSEPH J. BYERS, OF BROOKLINE, MASSACHUSETTS, ASSIGNOR TO PRODUCTS SYNDICATE, INC., OF BOSTON, MASSACHUSETTS, A CORPORATION OF MASSACHUSETTS.

## PROCESS OF TREATING MATERIALS WITH CELLULOSE DERIVATIVES.

1,388,169.

Specification of Letters Patent. Patented Aug. 23, 1921.

No Drawing.

Application filed April 19, 1916. Serial No. 92,320.

To all whom it may concern:

Be it known that I, JOSEPH J. BYERS, a citizen of the United States, and a resident of Brookline, county of Norfolk, State of Massachusetts, (whose post-office address is 26 Broad street, Boston, Massachusetts,) have invented an Improvement in Processes of Treating Materials with Cellulose Derivatives, of which the following description is 10 a specification.

This invention relates to methods of treating penetrable materials with a cellulose derivative, the object being to improve such materials with respect to certain desirable 15 qualities.

The invention will be best understood by reference to the following description which illustrates by way of example the application of one form of the process to a specific 20 case, while its scope will be more particularly pointed out in the appended claims.

The preferred manner of carrying out the method is to treat the material with a cement-like substance consisting of or including 25 a cellulose derivative in solution and containing a quantity of non-oxidizing oil, and the best results are apparently obtained by thoroughly impregnating the material with the cement and oil.

30 The materials comprising the cement and the proportions in which they are mixed may be varied within wide limits. A suitable cement, for example, may be prepared by dissolving some cellulose derivative, such 35 as a soluble nitro-cellulose, for example, celluloid, in a suitable solvent, which may be, for example, acetone and alcohol in equal parts; if, for illustration, celluloid and acetone and alcohol are used, one pound of 40 celluloid to one gallon of solvent may be employed with good results. To this is preferably added a substantial amount of some non-oxidizing or non-drying oil, preferably a vegetable oil. This, for example, may be 45 castor oil in the proportion of eight ounces to one gallon of solvent.

The preferred method of treatment is to immerse the material in a bath composed of the cement. For illustration, a bath may be 50 prepared of sufficient volume in proportion to the mass of the material to be treated to maintain the material immersed for the required time thoroughly to impregnate it without impairing the fluidity or effectiveness of the cement. The tank or other re-

ceptacle employed for the bath is preferably closed to prevent any substantial evaporation of the solvent during the treatment of the material, and is also preferably provided with suitably controlled heating means 60 so as to maintain the bath at a suitable temperature.

The temperature of the bath is preferably maintained at a point above the normal temperature of the air, but below that which would rapidly evaporate the solvent or impair the qualities of the oil or the material to be treated. In the treatment of leather with a cement constituted as described and containing the stated amount of castor oil, 70 the temperature should be preferably less than 160° F. Good results are had from temperatures varying from 125° to 130° F.

Porous materials such as leather usually hold absorbed more or less hygroscopic 75 moisture. To facilitate the impregnation of the material with the cement, it is preferable to remove substantially all water and hygroscopic moisture from the material before its treatment. This may be accomplished in any desired manner, but, in the case of leather, a simple method is to expose the material to a suitable drying temperature for a period long enough to drive out the moisture. The time and temperature 80 required will differ for different materials and different masses of the same material. In the case of sole leather, for example, the leather may be hung or spread over night in a drying room or drying oven at a temperature of from 120° to 150° F. In the case of some textile fabrics or thin sheet materials, the material may be prepared for immersion by passing the same slowly through a drying 85 room or drying apparatus. 90

Preferably also the material should be handled and the treatment carried out in a room where the air has a low humidity so that in passing from the drying operation to the immersion, the material may have no opportunity to absorb or collect any substantial or detrimental amount of moisture. While no particular temperature in the room where the operation is carried out is essential to the invention, good results are secured where it is maintained between 70° and 80° F. 105

By expelling substantially all of the moisture in the leather or other material and immersing it while in a dry state, the per- 110

meation or impregnation of the material is facilitated and it is possible to impregnate the entire mass with the cement, the non-oxidizing oil in the latter apparently replacing the moisture in the individual fibers or particles of the mass.

With the material dried as described, it may be immediately plunged into the bath and there maintained immersed in the presence of heat and the oil for a long enough period thoroughly to impregnate it with the oil and cement.

The period during which the immersion may be profitably continued will vary with the material and its thickness. For sole leather, for example, it may require from two to six hours, according to the thickness. In the case of some thin, permeable sheet material, a few minutes or less will sometimes suffice. Preferably the immersion is continued for an appreciable period sufficiently prolonged to impregnate the material throughout. In the presence of heat and immersed in the solution, the material soon becomes impregnated with the cement. In the case of fibrous material such as leather, the fibers, I believe, become charged with the oil with perhaps more or less cement, while at the same time they become coated over by and incased in the cement which permeates the entire mass.

After removing the material from the bath, it may then be dried. The effect of this is apparently to unite the fibers or particles into a homogeneous mass, leaving the oil sealed in the particles or fibers and protected by the cement which, as I believe, incases them and binds them together throughout. The material treated by this method may be thoroughly impregnated throughout as distinct from a mere surface coating or a coating which has an anchorage or impregnation of limited depth. Leather treated by this method acquires the property of repelling water, has great durability and density and a high degree of flexibility. Its water repellent properties, moreover, are long continuing, which I attribute to the fact that the oil which is sealed into the individual fibers or particles by the cement cannot be washed out by exposure to moisture. The fibers of the leather appear to have an oil-flexed property which is substantially permanent, while the oil commingled with the cement throughout the body gives it a high degree of permanent flexibility.

Before being thoroughly dried, the material, if desired, may be subjected to some action which will condense and compact the cement impregnated mass. While this step may be omitted and a useful product still produced, a superior product may be produced by subjecting it to pressure before completely drying. If it is desired to com-

pact the cement-impregnated material, the latter, after being removed from the bath, may be subjected to one or more pressing operations tending to press and bind the fibers more closely together. This pressing operation may be carried out in any desired manner, as, for example, in a press or by passing the material progressively between preferably heated rolls. In the case of leather, for example, it may be run between successive pairs of heated rolls, the members of successive pairs being separated by graduated distances so that the material is gradually compacted and rendered more dense, preventing its expansion when subjected to moisture.

In the case of some materials, as, for example, in the case of sole leather, a greater compactness may be secured by allowing the material partly to dry after removal from the bath, before compacting it. In such cases the leather or other material, after first having the excess of cement removed from its surface and after having been partly dried, the drying being carried far enough to set the cement at or near the surface, it may then be compressed between rolls or by any other suitable means. After being passed through a suitable number of compressing operations, the compressed cement-impregnated material is then thoroughly dried.

The cement-impregnated material may, if desired, be coated with one or more coatings of the cement solution or with any other suitable solution of a cellulose derivative either for the purpose of finishing the surface, or for any other purpose. For example, to surface-coat cement-impregnated leather, the latter after having been impregnated, compressed and dried, may then be surface-coated with a cement solution. This solution by way of illustration may be similar to that composing the bath. With the coating partly dried, it may then be run between hot compression rolls, and this operation may be repeated as many times as is desired.

In the case of leather, the product of this process is characterized by greater toughness, compactness and durability than the original leather before treatment and is substantially and permanently water-repellent. While tougher and more durable, it is highly flexible because of the oil-filled, cement-coated fibers. By this process durability, toughness, compactness and water-repellent qualities may be so imparted to cheap or inferior grades of leather as to make them available for uses and purposes not heretofore possible, and as equal or better substitutes for leather of more expensive grades.

In the case of leather, a product may be produced which while water-repellent is not

- wholly impervious to air, rendering it available for certain uses where some degree of porosity is desired and where such a material as rubber, for example, is undesirable.
- 5 Apparently the fibers become incased with the cement after the leather has been immersed without necessarily wholly filling the interstices between the fibers or wholly expelling the air from within the same. This
- 10 fibrocellular structure of the leather may be preserved to a greater or less extent according to the degree to which the compacting operation is carried.

15 The treatment of leather or textile materials by my process assists in preserving the same. When employed for footwear, for example, it resists the rotting action which, in the case of ordinary leather, is due in part to the presence of ammonia in the perspiration from the foot.

20 I do not herein claim the product which is herein described as produced by the disclosed method, the product being claimed in my co-pending application Ser. No. 141,664, now Patent No. 1,327,197.

25 While I have herein described for purposes of illustration the steps in detail by which one form of my process may be carried out, it is to be understood that the invention is not limited to the exact details specified, but may be varied within suitable limits without departing from the spirit thereof, and furthermore, that while I have illustrated the same with reference to the 30 treatment of leather, other fibrous materials and penetrable materials other than fibrous materials may be treated by my process with beneficial results.

Claims:

- 40 1. The method of improving penetrable material which consists in immersing the material in a cement bath consisting of a cellulose derivative in a suitable solvent and a non-oxidizing oil, maintaining the material 45 in said bath in the presence of heat until impregnated throughout with the oil and cement, removing the same from the bath, and drying the same.
2. The method of improving penetrable 50 material which consists in immersing the material while substantially free from moisture in a cement bath consisting of nitrocellulose in a suitable solvent and a non-oxidizing oil, said solvent being in sufficient 55 proportions and said bath being of sufficient volume in proportion to the mass of material to maintain the fluidity of the cement during the immersion of the material, maintaining the material in said bath in the 60 presence of heat for a sufficient time to cause the oil and cement to penetrate throughout the mass of material, removing the material from the bath and drying the same.
3. The method of improving penetrable 65 material which consists in removing sub-
- stantially all moisture therefrom, immersing it while still free from moisture in a cement bath consisting of a cellulose derivative in a suitable solvent and a non-oxidizing oil, maintaining the material in the presence of 70 heat for a sufficient time to cause the oil and cement to penetrate throughout the mass of the material, withdrawing it from the bath, and drying the same to set the cement.
4. The method of improving penetrable 75 material which consists in removing substantially all moisture therefrom, immersing it while still free therefrom in a cement bath consisting of a cellulose derivative in a suitable solvent and a non-oxidizing oil, 80 maintaining the material in said bath in the presence of heat for a sufficient time to cause the oil and cement to penetrate through the mass of material, compacting the mass further to unite the cemented particles, and drying the compacted mass.
5. The method of improving penetrable 85 material which consists in withdrawing hygroscopic moisture from the material, immersing it while free therefrom in a cement 90 bath consisting of a cellulose derivative in a suitable solvent and a non-oxidizing oil, maintaining the temperature of said bath at from 120° to 170° F., maintaining the material in said bath until thoroughly impregnated with said oil and cement, removing it 95 from the bath, and drying the same.
6. The method of improving penetrable sheet material which consists in drying the material to remove substantially all moisture 100 therefrom, immersing it while still dry and in a dry atmosphere in a cement bath consisting of nitrocellulose in a suitable solvent together with a non-oxidizing oil, maintaining the material in said bath for a sufficient 105 time to cause the oil and cement to penetrate throughout the mass of the material, maintaining the temperature of the bath during immersion at a point less than the boiling temperature of the solvent and above the 110 temperature of the surrounding atmosphere, said bath being of sufficient volume to maintain the immersion of the material during the period of treatment, compacting the mass by heat and pressure, and drying the 115 compacted mass to set the cement.
7. The method of improving penetrable 120 material which consists in immersing the material while substantially free from moisture in a cement bath consisting of nitrocellulose in a suitable solvent and in the proportions of one gallon of solvent to one pound of nitrocellulose and containing a non-oxidizing oil, maintaining the bath at a temperature of from 120° to 160° F., keeping the material in said bath until the oil and cement have penetrated throughout the mass of material, expelling the excess of cement, compacting the mass by heat and pressure, and drying the compacted mass.

8. The method of improving penetrable material which consists in immersing the material in a bath containing a solution of a cellulose derivative, maintaining the material in said bath in the presence of heat and a non-oxidizing oil until impregnated, withdrawing the same from the bath and partly drying to set the cement near the surface, compacting the partly dried material further to unite the particles thereof, and completely drying the same.
9. The method of improving sheet material which consists in impregnating the same throughout in the presence of heat with a cement having a cellulose derivative in solution and a non-oxidizing oil, and thereafter pressing the cement-impregnated sheet.
10. The method of improving material which consists in impregnating it in the presence of heat with a solution of a cellulose derivative and a non-oxidizing oil.
11. The method of improving material

which consists in immersing it in the presence of heat in a bath having a cellulose derivative in solution and a non-oxidizing oil.

12. The method of improving penetrable material which consists in immersing the material in a bath containing nitro-cellulose in solution and containing also non-oxidizing oil, heating said bath, maintaining the material in said heated bath until the same is thoroughly impregnated, and compacting the material when removed from the bath to compress and condense the impregnated body thereof before drying.

In testimony whereof I have signed my name to this specification in the presence of two subscribing witnesses.

JOSEPH J. BYERS.

Witnesses:

ROBERT H. KAMMLER,  
THOMAS B. BOOTH.